

## UNITED STATES PATENT OFFICE

2,069,626

## LUBRICANT COMPOUND

Theodore G. Roehner, Malverne, N. Y., assignor  
to Socony-Vacuum Oil Company, Incorporated,  
New York, N. Y., a corporation of New  
York

No Drawing. Application July 3, 1934,  
Serial No. 733,609

2 Claims. (Cl. 87—9)

This invention has to do with lubricant compounds, and more particularly with the class of lubricants known as slushing oils. Slushing oils are used for the protection of metals, either in the form of stock or fabricated articles, against the normal hazards of corrosion. For instance, finished articles, prior to storage, are coated with slushing oils to prevent rusting while in storage. Finished articles and finished and semi-finished stocks, destined for shipment by rail or by water, must be protected against the attack of moisture by a coating of slushing oil. Semi-finished stocks in process require this protection, particularly when the finish of the completed article is to be obtained merely by polishing or burnishing the surface of the stock. Particularly outstanding examples of this class are strip stock used in the manufacture of razor blades, which must be inspected literally inch by inch, and which must undergo such inspection and similar handling without retaining the inspectors' fingerprints, and cold rolled strip steel to be used for such things as the handles on electric irons, etc., which must likewise be free from the marks of handling or of other corrosion.

This invention has to do with the production of a novel slushing oil adapted for these various purposes and containing as a characterizing ingredient, a proportion of pine fatty acids. The invention is based upon the discovery that a slushing oil having new and advantageous properties not heretofore attained in this class of compounds can be produced by the use of pine fatty acids in the manner described below.

These pine fatty acids, which I have discovered to be useful for the purposes discussed herein, are apparently true fatty acids, obtained by fractional distillation of fatty matter separated from pine wood in the course of cooking by the alkaline process for the manufacture of wood pulp. As an indication of the nature of these compounds, I may give the following test data

Specific gravity @ 60/60° F. 0.90-1.00  
Moisture (ASTM xylol) 0.10%-0.30%  
45 Saponification value (ASTM) 150-170 mg. KOH  
Iodine value (Hanus) 40-150  
Titer of separated fatty acids (ASTM) 50-90  
Color (ASTM colorimeter) Dark 8 or lighter  
Saybolt universal viscosity @ 100° F. 100-600  
50 Flash (ASTM open cup) 250° F. Min.  
Free fatty acids (ASTM) 90% Min.  
Ash content (ignition) Trace-0.1%

From the above data it may be seen that these 55 "pine fatty acids" do not partake of the charac-

ter of other commonly used pine derivatives, but are true fatty acids. They are for instance quite distinct from the "pine oils" which are essentially terpene-like in character, and from rosin, which is essentially abietic acid of varying degrees of purity, abietic acid being of different properties from those indicated above.

I have found that a small proportion of these pine fatty acids, when blended with commercial mineral oil fractions of the proper kind, afford 10 an efficient protection of the metal treated, as for instance in the protection of razor blade stock from the corrosive action of fingerprints. Previously known slushing oils have usually been composed of such compounds as petrolatum 15 and/or mineral pitches, petroleum pitches and like compounds, diluted with kerosene, spindle oil, or light solvent oils. Frequently, use has been made of inorganic chromates dissolved in various mineral oils. A very popular class of prior 20 art slushing compounds has been composed of animal fats such as degras, wool fat, lanolin, talow oil, etc., dissolved in kerosene or similar solvents. An extremely popular compound of this kind has been anhydrous lanolin dissolved in a 25 proper mineral oil. The popularity of this compound has been due to an undoubted superiority over all other prior art compounds, which superiority has been generally accepted.

I have discovered that the use of pine fatty 30 acids in the manner described herein gives rise to slushing oils greatly superior to the lanolin compounds. As an example of the superiority of the slushing compounds made according to this invention, over lanolin slushing oils, I may 35 cite the fact that, in a commercial plant engaged in the manufacture of razor blades, and using a slushing compound composed of anhydrous lanolin and mineral oil, it was necessary for the workmen to keep their hands very heavily powdered with moisture-absorbing powder, and even with these precautions, there was a fairly high rejection rate on fingerprinted razor blade stock. Upon replacing the old style slushing oil with one containing pine fatty acids in accordance 45 with this invention, the rejection rate due to fingerprinting dropped nearly to zero. As a matter of fact, numerous tests have indicated that under ordinary commercial conditions, it is probably entirely possible to handle razor blade stock 50 which has been slushed with my preferred compound, without even the precaution of powdering the hands. As a further example of the efficacy of these compounds for the protection of metals against corrosion, the handling of cold 55

rolled strip steel and shipment of it by barge for a considerable distance coastwise may be mentioned. The stock was slushed prior to packing, with a compound of mineral oil and 5 semi-refined degras which the manufacturer had found by previous experience to be the most effective for his use of the slushing oils available upon the market. It was packed at the waterfront under what might be described as conditions 10 very desirable for salt-air corrosion, and was placed in boxes lined with paraffin paper. The rejection rate of corroded stock was fairly high as the finishing operation was merely a buffing of the surface of the stock after forming 15 into flat iron handles. Upon substituting for the old slushing oil, a new slushing oil containing pine fatty acids in accordance with this invention, and without changing any of the other conditions, the rejections due to corrosion dropped 20 practically to zero.

It is my belief that this superior protective ability inherent in slushing oil compounds prepared with pine fatty acids according to this invention, is due to the wetting characteristics 25 of these compounds. The slushing oil so compounded appears to so wet the steel that it is not ordinarily displaced by perspiration or atmospheric moisture, or corrosive agents of similar nature.

30 As an example of one preferred formula which I have found applicable for the above purposes, namely, those of protecting metals against the corrosive attack of moisture, etc., I present:

| Ingredient                | Per cent |
|---------------------------|----------|
| Pine fatty acids          | 3        |
| Light paraffin oil        | 48       |
| Kerosene                  | 48       |
| Steam distillate pine oil | 1        |

35 In this formula the pine oil ingredient is present for the purpose of lending an agreeable odor. Another formula I have found to be widely applicable is:

| Ingredient         | Per cent |
|--------------------|----------|
| Pine fatty acids   | 3.4      |
| Amber petrolatum   | 11.4     |
| Light paraffin oil | 85.2     |

The characteristics of the slushing compound desired are determined largely by the nature of and intended destination of the material to be protected by such slushing oils. For instance, the manufacturer of razor blades who desires to protect his product during intermediate processing, usually wants a protective film of the maximum thinness and "hardness" consistent with the protection obtained, while as an opposite extreme, the manufacturer who is shipping a heavy assembled piece of machinery overseas might desire a slushing compound which will not only give an extremely thick protective film, but which will be somewhat of the nature of a grease and have some lubricating properties, so that it need not be disturbed when the machinery is placed

in operation, but might be gradually displaced by the lubricant used. To obtain the light, thin "hard" film desired in cases of interprocess protection, it is preferred to blend the pine fatty acids with such material as kerosenes and extremely light lubricants in varying proportions. To obtain the heavy slushing oils, it is preferred to use increasing percentages of petrolatum or similar body-giving ingredients, and compounds of all desired consistencies between these two extremes may be obtained by varying the nature and character of the ingredients. It is even desirable in certain cases, to use animal fats in the slushing oil compound, such as lanolin or degras, and similar fats, or to use vegetable fats such as japan wax or similar fats, or even to use waxes of various origins, such as paraffin wax, or carnauba wax. Experimentation has developed the fact that the effective range for the concentration of pine fatty acids in such slushing oils is probably 20 between 1% and 5% of the total compound, with an indicated maximum effective balance of protective ability and cost at around 3%. The range of compositions indicated for these slushing oils is probably best expressed by the following tabulation:

| Ingredient         | Range |      | Preferred for |       |
|--------------------|-------|------|---------------|-------|
|                    | Min.  | Max. | Light         | Heavy |
| Pine fatty acids   | 1     | 5    | 1-3           | 1-3   |
| Light paraffin oil | 0     | 99   | 30-60         | 99-50 |
| Kerosene           | 0     | 99   | 60-30         |       |
| Petrolatum         | 0     | 50   |               | 0-50  |

In case vegetable fats, animal fats, or waxes are added to the composition, they may generally be present in amounts up to about 20% of the total and the primary mixture to which they are added may be any of the above indicated mixtures, as dictated by the conditions of use. The method of compounding these slushing oils is merely one of physical admixture of the various ingredients.

I claim:

1. An oil composition for application to metal surfaces to protect them from corrosion incidental to handling, inspection, or normal exposure, by forming a coating notably resistant to displacement by moisture, comprising a mineral oil distillate, petrolatum, and pine fatty acids.

2. An oil composition for application to metal surfaces to protect them from corrosion incidental to handling, inspection, or normal exposure, by forming a coating notably resistant to displacement by moisture, comprising

| Ingredient         | Per cent |
|--------------------|----------|
| Pine fatty acids   | 3 to 5   |
| Amber petrolatum   | 8 to 15  |
| Light paraffin oil | 89 to 80 |

THEODORE G. ROEHRER.